

## UNITED STATES PATENT OFFICE.

HENRY C. PRITHAM, OF UPPER DARBY, PENNSYLVANIA.

## TRACER COMPOSITION.

No Drawing.

Application filed May 23, 1924. Serial No. 715,457.

(GRANTED UNDER THE ACT OF MARCH 3, 1883, AS AMENDED APRIL 30, 1928; 370 O. G. 757.)

The invention described herein may be manufactured and used by or for the Government or for governmental purposes without the payment to me of any royalty there-

5 on.

The subject of this invention is a combustible composition or mixture burning with greater or less rapidity, as may be desired, and possessing the desirable quality 10 of luminosity, brilliance, or visibility in burning; the mixture being especially adapted for use as a tracer mixture in projectiles, though also useful in many other organizations, such as port fires, rockets, signal fires, 15 and any burning composition in which the above mentioned qualities are desirable.

It has been found that the addition of certain rare earth elements to combustible materials will greatly increase the luminosity, brilliance and visibility thereof 20 when combustion takes place. These same elements, or proper salts thereof, when themselves combustible, may be used either alone or in combination with other elements for 25 the purpose above outlined.

While any rare earth element possessing the characteristics, when heated, of giving off an unusually large proportion of its energy in the form of light waves are adapted 30 to produce the above outlined desired results; the preferred elements for this purpose are thorium and cerium.

These elements may be used either in the 35 form of a nitrate or other oxygen carrier; in the form of a fuel, as a sulpho-cyanates; or in the form of inert substances merely for increasing the brilliance, as in oxide or chloride.

The following tracer mixtures are typical examples of different uses of these elements: 40

As an oxygen carrier:

|                   | Parts. |
|-------------------|--------|
| Strontium nitrate | 60     |
| Cerium nitrate    | 40     |
| Thorium nitrate   | 1.1    |
| Magnesium         | 40     |
| Calcium resinate  | 25     |

As an inert substance:

|                   | Parts. |
|-------------------|--------|
| Strontium nitrate | 50     |
| Sodium nitrate    | 60     |
| Magnesium         | 40     |
| Calcium oxide     | 20     |
| Thorium oxide     | 10     |
| Cerium oxide      | 10     |

The following are typical examples of combustible mixtures of the salts.

|                      |                |
|----------------------|----------------|
| Thorium-cerium salts | 90 to 98 parts |
| Thorium salts        | 2 to 10 " or   |
| Thorium salts        | 90 to 98 " 60  |
| Cerium salts         | 2 to 10 "      |

While the above mixtures are typical tracer mixtures they are cited only by way of example and are intended in no way to limit the proportions of the various ingredients to those set forth as the proportions in which the thorium or cerium salts will be used depend largely upon the other ingredients mixed therewith and the use to which the mixture is intended to be put.

Having thus described the invention what is claimed is:

1. A non-explosive pyrotechnic composition including as elements salts of thorium and cerium and a binder.

2. A tracer composition for projectiles including nitrates of an alkali earth metal, salts of cerium and thorium, a fuel and a binder.
3. A tracer composition for projectiles including nitrates of alkali earth metals, an oxide of an alkali earth metal, salts of cerium and thorium a fuel and a binder.
4. A tracer composition for projectiles including nitrates of alkali earth metals, an oxide of an alkali earth metal, salts of rare earth metals a fuel and a binder.
5. A tracer composition for projectiles including nitrates of an alkali earth metal, sulphocyanates of cerium and thorium a 15 fuel and a binder.
6. A tracer composition for projectiles including nitrates of an alkali earth metal, salts of cerium and thorium and a fuel.
7. A tracer composition for projectiles, in- 20 cluding strontium nitrate 60 parts, magnesium 40 parts, cerium thorium salts, 41 parts, calcium resinate 45 parts.

HENRY C. PRITHAM.